

## UNITED STATES PATENT OFFICE

2,211,798

## OIL COMPOSITION

Bertrand W. Story, Wenonah, and Everett W. Fuller, Woodbury, N. J., assignors to Socony-Vacuum Oil Company, Incorporated, New York, N. Y., a corporation of New York

No Drawing. Application March 2, 1937.  
Serial No. 128,601

## 4 Claims.

(Cl. 87—9)

This invention relates to the stabilization, against the effects of atmospheric oxygen, of viscous petroleum oils, such as transformer oils and technical white oils, which are of a highly refined character and substantially free from unsaturated hydrocarbons and resinous compounds.

Oils of the kind in question are commonly made by refining petroleum distillates of the requisite viscosity by treatment with large quantities of sulphuric acid, including fuming acid, followed by neutralization and clay filtration or redistillation. So far as the present invention is concerned, however, the method by which the highly refined character is imparted to the oils is unimportant.

It is well known that highly refined viscous petroleum oils, although very stable against oxidation at atmospheric temperatures, tend to absorb atmospheric oxygen when heated, particularly when in contact with catalytic metals such as copper, and that the first result of such oxidation is the production of acid compounds soluble in the oils. The oils thereby become unsuitable for the uses to which they are chiefly applied, that is, as transformer oils, turbine lubricants and the like, and must be purified or replaced.

It is known that both elementary sulphur and various organic sulphur compounds have the power of stabilizing oils, including some petroleum oils, in some degree against atmospheric oxidation, but sulphur and the sulphur compounds previously known to have this power have been practically useless for the purpose of stabilizing oils of the type here referred to, because they are either corrosive to copper and other metals in contact with which the oils are used, or not sufficiently soluble in the oils to permit the use of a quantity great enough for effective results.

In our application filed June 10, 1931, Serial No. 543,398, of which the present application is a continuation in part, we have disclosed the discovery that organic disulphides, as a class, have the power, when dissolved in highly refined viscous petroleum oils, of inhibiting, in varying degrees, the oxidation of such oils under the conditions of use, and that such disulphides have little or no tendency to attack copper. These disulphides, however, vary widely in their effectiveness, owing to differences in solubility or to other causes not definitely known, so that some of them would be of little commercial utility as compared with other known materials for the same purpose.

We have discovered that a sub-class of organic

disulphides which are particularly effective are those in which the sulphur atoms are united directly with groups or radicals other than benzene rings, particularly alkyl radicals and thiuram and thiazo groups, these particular sulphides being relatively soluble in the oils and being, in all cases investigated, sufficiently effective for commercial use.

The foregoing applies both to the simple alkyl disulphides, such as diethyl disulphide and di-n-butyl disulphide, and to the aralkyl disulphides, such as dibenzyl disulphide, in which aryl groups are substituted for one or more hydrogen atoms of the intermediate alkyl groups. On the other hand, we have found that aromatic disulphides, in which the rings are directly connected to the sulphur, are relatively ineffective.

The effectiveness of stabilizers of the kind in question may be evaluated not only by actual use of the stabilized oils in transformers and machinery, but also by a laboratory test, commonly known as the "German tar test," which has been found to give results comparable in degree with the results in actual use. In accordance with this method, a weighed sample of the oil is maintained at a temperature of 120° C. and oxygen gas bubbled through it slowly for 70 hours. The sample is then extracted with alcoholic soda solution, and the extracted material is precipitated by means of an acid, and dried and weighed. The weight of the precipitate or acid extract varies directly with the susceptibility of the oil to acid formation under the conditions of the test.

In the tests specifically described herein, the oil used was a highly refined viscous petroleum oil containing paraffines and naphthenes but substantially free from unsaturated hydrocarbons and resinous bodies. The oil, in the absence of stabilizers, was readily susceptible to oxidation, as it yielded an acid extract, under the test described, of approximately 14%.

The following table shows the results when the said oil was tested with various alkyl, aralkyl and thiazo disulphides, in optimum quantities:

| Disulphide           | Quantity | Acid extract | 45 |
|----------------------|----------|--------------|----|
| Percent              | Percent  |              |    |
| Diethyl              | .10      | .02          |    |
| Di-n-butyl           | .10      | .02          | 50 |
| Di-isooamyl          | .05      | .07          |    |
| Dibenzyl             | .05      | .08          |    |
| Di-phenyl ethyl      | .05      | .03          |    |
| Di-phenyl n-propyl   | .05      | .04          |    |
| Benzothiazole        | .05      | .08          |    |
| Tetra-methyl thiuram | .03      | .03          |    |

55

Tetramethyl thiuram disulfide is a dithiocarbonic acid derivative having the formula



which, it will be observed, contains the characterizing group



For comparison with the foregoing, tests made on the same oil, in the same way, showed that with the addition of .10% of diphenyl disulphide the acid extract was reduced only to 5.1%, while with the maximum soluble quantity of diphenyl disulphide, somewhat less than .10%, the acid extract was reduced only to 13.0%.

For commercial use, under present conditions, we have found dibenzyl disulphide the most suitable of the antioxidants herein disclosed, owing to its effectiveness, relatively low cost and high boiling point. It usually has its optimum effect in a quantity of not over 0.10%, but in a quantity of only 0.01% it has been found to reduce, by more than one half, the acid extract produced in testing the oil used in the foregoing tests.

We claim as our invention:

1. The combination, with a highly refined viscous petroleum oil, of material selected from the class of disulphides consisting of the alkyl disulphides, the aryl-substituted alkyl disulphides and the thiuram and thiazo disulphides, in a quantity sufficient to diminish substantially the production of acidic compounds in the oil as the result of atmospheric oxidation at elevated temperature. 5

2. The combination, with a highly refined viscous petroleum oil, of an alkyl disulphide, in a quantity sufficient to diminish substantially the production of acidic compounds in the oil as the result of atmospheric oxidation at elevated temperature. 10

3. The combination, with a highly refined viscous petroleum oil, of tetra-methyl thiuram disulphide, in a quantity sufficient to diminish substantially the production of acidic compounds in the oil as the result of atmospheric oxidation at elevated temperature. 20

4. The combination, with a highly refined viscous petroleum oil, of benzothiazole disulphide in a quantity sufficient to diminish substantially the production of acidic compounds in the oil as the result of atmospheric oxidation at elevated temperature. 25

BERTRAND W. STORY. 30  
EVERETT W. FULLER.

CERTIFICATE OF CORRECTION.

Patent No. 2,211,798.

August 20, 1940.

BERTRAND W. STORY, ET AL.

It is hereby certified that error appears in the printed specification of the above numbered patent requiring correction as follows: Page 1, first column, line 10, for "suphuric" read --sulphuric--; line 41, for "543,398" read --543,396--; and second column, line 53, in the table, for "Benzothiazole" read --Benzothiazole--; and that the said Letters Patent should be read with this correction therein that the same may conform to the record of the case in the Patent Office.

Signed and sealed this 25th day of February, A. D. 1941.

(Seal)

Henry Van Arsdale,  
Acting Commissioner of Patents.

CERTIFICATE OF CORRECTION.

Patent No. 2,211,798.

August 20, 1940.

BERTRAND W. STORY, ET AL.

It is hereby certified that error appears in the printed specification of the above numbered patent requiring correction as follows: Page 1, first column, line 10, for "suphuric" read --sulphuric--; line 41, for "543,398" read --543,396--; and second column, line 53, in the table, for "Benzothial-azole" read --Benzothiazole--; and that the said Letters Patent should be read with this correction therein that the same may conform to the record of the case in the Patent Office.

Signed and sealed this 25th day of February, A. D. 1941.

(Seal)

Henry Van Arsdale,  
Acting Commissioner of Patents.